

Patented Mar. 13, 1923.

1,448,246

# UNITED STATES PATENT OFFICE.

EDWARD GOODRICH ACHESON, OF NEW YORK, N. Y.

## LUBRICATING OIL.

No Drawing.

Application filed August 28, 1919. Serial No. 320,519.

To all whom it may concern:

Be it known that I, EDWARD G. ACHESON, a citizen of the United States, residing at New York, in the county of New York and 5 State of New York, have invented certain new and useful Improvements in Lubricating Oils, of which the following is a specification.

This invention relates to a novel lubricating oil having the essential and characteristic lubricating properties of an unfiltered oil-distillate of lubricating grade, but modified or standardized as to color and appearance by the addition thereto of a deflocculated or 15 colloidal solid material which does not substantially affect the lubricating properties of the oil. The invention relates also to the method whereby the novel lubricating oil is prepared.

As is well known to those familiar with this art, the manufacture of the so-called high-grade lubricating oils involves a number of relatively costly and at times troublesome, difficult and wasteful process steps and 25 treatments which follow the condensation and recovery of the raw distillate of lubricating grade. While these treatments may vary somewhat in accordance with the practice of individual producers, all of them, so far as I 30 am aware, include a treatment of the raw distillate (by which term I designate the condensate of lubricating grade as derived from the stills) with sulfuric acid, followed by neutralization with caustic soda and an elaborate washing process; and a so-called filtration which is in effect a treatment with 35 fuller's earth or equivalent decolorizing agent.

Comparative studies of the true lubricating value of the oil at the various stages of 40 its manufacture have shown that in many cases at least the lubricating value of the original crude distillate is very materially in excess of that of the filtered oil which is distributed to the consumer. Also, so far as I 45 am aware, the actual effect of the so-called filtration, or fuller's earth treatment, is in practically every case to bring about a decided and material diminution of the lubricating value of the oil, owing to the removal 50 of constituents, presumably colloidal in nature, which contribute to the production and proper maintenance of the most desirable lubricating film.

The primary purpose and effect of the 55 treatment steps to which the crude distillate

is subjected in the current manufacturing operations, is therefore to improve the color and appearance of the oil, and to some extent to improve its odor. So far as the filtering operation is concerned, practically its only purpose and effect is to improve the appearance of the oil, and to produce a bright oil of light color, which is commonly altho of course erroneously, believed to be 60 "free from carbon" and hence less liable to lead to carbonization difficulties when used in internal combustion motors.

A primary object of the present invention is to produce a salable product having a 70 standardized and attractive color and appearance, while retaining to the fullest degree the essential and characteristic lubricating qualities of the unfiltered distillate, or of the raw distillate in those cases in which 75 the lubricating value of the raw distillate is equal to or greater than that of the refined distillate. In other words, in accordance with this invention the treatment of the oil is related to its use as a lubricant, and to the 80 conservation of the full lubricating value of the raw distillate, instead of with sole reference to the appearance of the oil as is the present practice.

I add to the unfiltered distillate, which 85 may be the raw distillate in the case of those oils in which the acid and alkali treatment does not enhance the lubricating value, a minute proportion of a deflocculated solid body. For example lamp-black gas-black, 90 or other form of amorphous carbon, deflocculated or transformed to the colloidal state by treatment with tannin or its equivalents in accordance with methods described in my prior patents and now well understood in 95 the art, and thereafter suspended in the unfiltered distillate in proportions amounting to only a few thousandths of one per cent by weight of the distillate, imparts to the oil, irrespective of its original color, a uniform black appearance, opaque by reflected light, although semi-transparent or translucent by transmitted light when the proportion of deflocculated lamp black is sufficiently small. Other effects may be obtained by a choice 100 of other deflocculated solids, among which I may mention clay, graphite, aluminum powder of the kind used for aluminum paints, etc. The proportion of such deflocculated bodies required to standardize the 105 appearance of the distillates is so very minute (seldom exceeding 0.1% by weight of

distillate and often as low as 0.005% that it is not necessary as a rule to consider whether the solid material is in itself a lubricant, although a substance of lubricating qualities, such for example as graphite, will naturally be preferred in many cases.

The present invention is specifically distinguished from that of my prior patents relating to the improvement of the lubricating qualities of oils by the suspension therein of deflocculated graphite, in that it contemplates the employment of deflocculated solids irrespective of their lubricating qualities, added to the unfiltered distillate in such proportions as will not materially modify the characteristic lubricating qualities of the distillate.

I claim:

- 20 1. A lubricating oil having the composition and essential characteristics of unfiltered distillate of lubricating grade, and a standardized color and appearance due to the addition thereto of a minute proportion of a deflocculated body.
- 25 2. A lubricating oil having the composition and essential characteristics of unfiltered distillate of lubricating grade, and a standardized black color and appearance

due to the addition thereto of a minute proportion of deflocculated carbon. 30

3. A lubricating oil having the composition and essential characteristics of unfiltered distillate of lubricating grade, and a standardized color and appearance due to the addition thereto of a deflocculated body 35 in proportion not exceeding 0.1% by weight of the oil.

4. A lubricating oil having the composition and essential characteristics of unfiltered distillate of lubricating grade, and a 40 standardized color and appearance due to the addition thereto of a deflocculated carbon in proportion not exceeding 0.1% by weight of the oil.

5. Method of standardizing distillates of 45 lubricating grade containing constituents removable by filtration, comprising adding thereto a deflocculated body in minute proportion.

6. Method of standardizing distillates of 50 lubricating grade containing constituents removable by filtration, comprising adding thereto a deflocculated body in proportion not exceeding 0.1% by weight of the oil.

In testimony whereof, I affix my signature. 55  
EDWARD GOODRICH ACHESON.